

# United States Patent Office

2,856,330

Patented Oct. 14, 1958

1

2,856,330

## METHOD OF TREATING COTTON FABRICS

Harold N. Vagenius, Chicago, Ill.

No Drawing. Application November 8, 1954  
Serial No. 467,658

4 Claims. (Cl. 167—84)

This invention relates to methods of treating cotton fabrics for preventing or delaying the development of unpleasant odors and/or a rise in pH value when the treated fabrics are exposed to or impregnated with body secretions such as perspiration or urine. The methods of this invention are particularly applicable to the treatment of diapers for the indicated purpose.

The methods of this invention involve dipping or submerging cotton fabrics in dilute water solutions of copper salts. However, such treatment of cotton fabrics ordinarily or often causes the fabrics to be tinted green, especially in the presence of small amounts of colloidal materials such as soaps, gums, starches, proteins such as albumen or casein and other colloidal material used in washing or treating fabrics and apt to remain in the fabrics after washing or treatment therewith. Further, dipping or submerging cotton fabrics in dilute water solutions of copper salts often render the fabrics water repellent.

It is, therefore, an object of the present invention to provide methods for treating cotton fabrics with dilute water solutions of copper salts without tinting the fabrics green or rendering the fabrics water repellent, even when the fabrics or the dipping solution of the copper salts contain colloidal materials such as soap.

According to the present invention, cotton fabrics are immersed in water solutions of a water soluble copper salt such as copper sulfate, chloride, acetate or nitrate. From about 0.05 to about 1 milligram molecules (an amount in milligrams numerically equal to the molecular weight) of copper salt are used for each 60 grams of cotton fabric. This amount of copper salt is dissolved in from 100 cc. to 1000 cc. or more of water. Further, from about 2 to about 10 milligram molecules of disodium dihydrogen pyrophosphate are added to the solution for each milligram molecule of copper salt. Also, the pH of the dipping solution is kept acid, preferably at a pH of from about 3.0 to 3.5 to about 5 or 6. The time of immersion may be from 1 or 2 minutes up to 10 or 15 minutes or longer, but is not critical. The immersion may be carried out at room temperature or at elevated temperatures for instance 120° F., or 140° F. or 160° F.

The above mentioned pH range is most suitably maintained by adding to the dipping solution appropriate amounts of acidic substances such as zinc or magnesium silicofluoride, acetic acid, lactic acid, hydrochloric acid, sulfuric acid and the like. In place of the disodium dihydrogen pyrophosphate, equivalent amounts of tetrasodium pyrophosphate may be used, but then an additional amount of an acidic substance is added to neutralize one half of the sodium content of the tetrasodium pyrophosphate. In place of the sodium pyrophosphate, other alkali metal pyrophosphates may be used, such as the corresponding potassium pyrophosphates.

For convenience in making up the dipping solution, mixtures may be prepared comprising a finely divided copper salt and finely divided disodium dihydrogen pyrophosphate in a ratio of one molecule of copper salt to two

2

to 10 molecules of said pyrophosphate. To insure proper acidity of the dipping solution, even in the presence of soaps, such mixtures may additionally comprise from one-half to two or more molecules of zinc or magnesium silicofluoride or equivalent acidic buffers for each molecule of said copper salt.

When cotton fabrics are treated as described in the preceding paragraph, then rinsed with water and dried, the fabrics are not rendered water repellent, nor are the fabrics tinted green, even when the fabrics (or the dipping solutions) contain even fairly large amounts of colloidal materials such as soaps, fats, oils, proteins such as albumen or casein, dirt or soil and the like. Further, cotton fabrics so treated contain copper substantively fixed thereon, which copper is not removed by wetting or rinsing with water or exposure to body secretions such as perspiration or urine. Further, fabrics so treated do not develop unpleasant odors and/or a rise in pH value and/or formation of ammonia when the treated fabrics are exposed to or impregnated with body secretions such as perspiration and urine.

Examples of treatments of 60 gram cotton diapers according to the present invention are given hereinbelow.

For each of these examples, one 60 gram cotton diaper was first wetted with 150 to 180 cc. water having .2 gram of ordinary soap dissolved therein, thereafter immersed for from three to ten minutes in a copper salt solution containing disodium dihydrogen pyrophosphate, then removed from the copper salt solution, squeezed thoroughly, rinsed with water and dried. The copper salts employed were the sulfate, chloride, acetate and nitrate. The pH was adjusted downwardly with an appropriate amount of zinc silicofluoride. The exact amounts of copper salts, pyrophosphate, water and the pH are tabulated as follows:

| Example No. | Copper Salt | Milligram Molecules of copper salt | Water, cc. | Milligram Molecules of pyrophosphate | pH  |
|-------------|-------------|------------------------------------|------------|--------------------------------------|-----|
| 40          | Sulfate     | 0.05                               | 250        | .1                                   | 5.0 |
| 1           | do          | 0.1                                | 250        | .2                                   | 4.5 |
| 2           | do          | 0.1                                | 250        | .3                                   | 4.5 |
| 3           | do          | 0.1                                | 250        | .4                                   | 3.5 |
| 4           | do          | 0.1                                | 250        | 2.0                                  | 3.5 |
| 5           | do          | 0.5                                | 350        | 5.0                                  | 3.5 |
| 6           | do          | 1.0                                | 450        | 10.0                                 | 3.5 |
| 7           | do          | 1.5                                | 550        | 0.3                                  | 3.5 |
| 45          | Chloride    | 0.1                                | 250        | 0.3                                  | 3.5 |
| 8           | Acetate     | 0.1                                | 250        | 0.3                                  | 3.5 |
| 9           | Nitrate     | 0.1                                | 250        | 0.3                                  | 3.5 |
| 10          | Nitrate     | 0.1                                | 250        | 0.3                                  | 3.5 |

An untreated diaper and each one of diapers Numbers 50 1 through 10 of the above table was impregnated with 90 cc. urine and placed in a polyethylene bag, which was kept at room temperature for six days. The control (untreated) diaper developed an unpleasant sour odor within 24 hours followed shortly thereafter by a rise in pH and generation of ammonia. In the case of diapers of Examples 1 through 10, such odor and rise in pH value did not take place before four or five days, and generation of ammonia did not occur at all.

Many details may be varied without departing from the 60 principles of this invention. It is therefore not my intention to limit the patent granted on this invention otherwise than necessitated by the scope of the appended claims.

I claim:

1. A method of treating cotton fabrics which comprises immersing said fabrics in a dilute acidic aqueous solution of a water soluble copper salt selected from the group consisting of the sulfate, chloride, nitrate and acetate, said solution containing, for each 60 grams of fabric, from about 100 to about 1000 cc. of water, from 65 about 0.05 to about 1 milligram molecules of a soluble copper salt, and from about 2 to about 10 milligram molecules of a di-alkali metal dihydrogen pyrophosphate

for each milligram molecule of said copper salt said solution being maintained at a pH of from about 3 to about 6.

2. A method according to claim 1 in which said pyrophosphate is a sodium pyrophosphate.

3. A method according to claim 1 in which said copper salt is copper sulfate.

4. As a new composition of matter, a mixture comprising a water soluble copper salt selected from the group consisting of the sulfate, chloride, nitrate and acetate and disodium dihydrogen pyrophosphate in a ratio of one molecule of said copper salt to from two to ten molecules of said pyrophosphate.

References Cited in the file of this patent

UNITED STATES PATENTS

|           |             |               |
|-----------|-------------|---------------|
| 22,362    | Glynn       | Dec. 21, 1858 |
| 43,233    | Stacey      | June 21, 1864 |
| 152,903   | Gender      | July 14, 1874 |
| 1,903,041 | Hall et al. | Mar. 28, 1933 |

|             |           |               |
|-------------|-----------|---------------|
| 1,960,627   | Finlayson | May 29, 1934  |
| 2,086,867   | Hall      | July 13, 1937 |
| 2,241,580   | Bishop    | May 13, 1941  |
| 2,580,286   | Dorsett   | Dec. 25, 1951 |
| 5 2,643,969 | Mahon     | June 30, 1953 |

FOREIGN PATENTS

|         |        |              |
|---------|--------|--------------|
| 453,348 | France | Apr. 2, 1913 |
|---------|--------|--------------|

OTHER REFERENCES

Fargher: Inhibitory Action of Certain Substances on the Growth of Mould Fungi, J. Text. Inst., vol. 21, 1930, pp. T245-T260.

15 Furry: Mildew-Resistant Treatments on Fabrics, Ind. and Eng. Chem., April 1941, pp. 538-545.

Fullerton: Cotton Duck and Canvas, Rot-proofing, J. Text. Inst., 1942, p. A321.

Textile Colorist, January 1943, p. 30.

20 Goodman: Cosmetic Dermatology, McGraw-Hill Book Co., 1936, p. 45, entry "Cupric Sulfas."